

No. 893,363.

PATENTED JULY 14, 1908.

W. PETERS & C. M. CASPERSSON.  
PROCESS OF CASTING METALS.  
APPLICATION FILED AUG. 23, 1907.

Fig. 1.



Fig. 2.

Inventors

W. Peters and  
Clas M. Caspersson

Witnesses

A. H. Rabraig,  
R. H. Butler

By

H. C. Everett & Co.

Attorneys

# UNITED STATES PATENT OFFICE.

WILLIAM PETERS AND CLAS M. CASPERSSON, OF MONESSEN, PENNSYLVANIA.

## PROCESS OF CASTING METALS.

No. 893,363.

Specification of Letters Patent.

Patented July 14, 1908.

Application filed August 23, 1907. Serial No. 389,870.

*To all whom it may concern:*

Be it known that we, WILLIAM PETERS, citizen of the United States of America, and CLAS M. CASPERSSON, a subject of the King 5 of Sweden, residing at Monessen, in the county of Westmoreland and State of Pennsylvania, have invented certain new and useful Improvements in Processes of Casting Metals, of which the following is a specification, reference being had therein to the accompanying drawing.

This invention relates to a process of casting metals, and its object is to produce metallic castings of superior quality by the 15 utilization of compressed air, oxygen or other fluid under pressure.

Another object of this invention is to prevent the splitting or "piping" of a casting or ingot.

20 It is a well known fact that in the process of cooling a casting or ingot, two important actions take place. First, there occurs what is known as a segregation of the material; that is to say, certain of the constituents of 25 the steel, such as carbon, phosphorus, and other impurities being of lighter specific gravity, tend to separate out from the mass and gather towards the top of the casting or ingot. Also, since the metal cools from the 30 outside towards the center, there is a tendency of the solidifying metal to shrink towards the outer surface and this causes a cup-shaped depression at the top of the ingot or casting, which extends down in the 35 form of a narrow slit or crack into the body of the metal, which, together with gas bubbles, forms which is known as "pipes." It is therefore apparent that the upper portion of the ingot or casting, because of its segregation or "piping," is less pure, more brittle, and as in the case of an ingot, is subject after 40 rolling to contain longitudinal flaws. It has been the practice to crop off approximately twenty-five per cent. of the ingot and 45 use the remaining part for the article to be produced by rolling.

By our improved process, we aim to prevent the segregation and rapid cooling of an ingot, and with a casting, we use sufficient metal 50 to prevent a "pipe" from being formed in the body of the casting, allowing the same

if it is formed to occur in a crop form upon the end of the casting.

The process consists in pouring molten metal into a suitable mold, and then subjecting the molten article to a blast of compressed air or other fluid to solidify the same. 55

In the accompanying drawings, Figure 1 is a vertical sectional view of a mold employed in carrying out our improved process, 60 Fig. 2 is a plan of the same.

The reference numeral 1 designates the body of the flask or mold, surmounted by a head-box 2. The flask 1 is adapted to contain sand or similar material, as indicated at 65 3, to receive a pattern, while in the head-box 2 is placed sand 4 to provide a gate 5. After the removal of the form or pattern, molten metal is poured into the flask to form the product 6, after which the molten article is 70 subjected to a blast of air or oxygen under pressure.

The reference numeral 7 designates a suitable blow pipe or nozzle protruding into the head-box 2 to subject the top of the molten 75 product to the action of air or a similar fluid under pressure. It will be observed that an excess amount of molten metal is used to produce the product 6, and that this metal forms a crop 8 in the head-box 2, and when said box 80 is removed, the crop can be sawed off.

The blast of air striking the top of the molten metal increases its solidification, and the density of the finished product, preventing segregation from taking place in the body of 85 the product 6 and thereby producing an article of greater strength, density and durability.

Having now described our invention what we claim as new is:—

A method of casting comprising the forming 90 of the product with a removable crop having a neck from sufficient metal to prevent the body of the product from piping, and then subjecting the crop prior to the cooling thereof to a blast of fluid under pressure. 95

In testimony whereof we affix our signatures in the presence of two witnesses.

WILLIAM PETERS.  
CLAS M. CASPERSSON.

Witnesses:

G. SPIEGELBERG,  
Wm. H. ZELLERS, Jr.